# EUROPEAN PATENT SPECIFICATION

(11) **EP 4 636 149 B1**
(45) Date of publication and mention of the grant of the patent: **29.07.2026**
(21) Application number: 24181777.4
(22) Date of filing: 12.06.2024
(51) Int. Cl.: D06C 3/02, D04H 1/46, D04H 1/492, D04H 1/56, D04H 3/16

(54) **METHOD FOR MANUFACTURING A NON-WOVEN FABRIC WITH ELASTICITY IN WARP DIRECTION**
VERFAHREN ZUR HERSTELLUNG VON EINEM VLIESSTOFF MIT ELASTIZITÄT IN KETTRICHTUNG
PROCÉDÉ DE FABRICATION D'UN TISSU NON TISSÉ PRÉSENTANT UNE ÉLASTICITÉ DANS LE SENS DE LA CHAÎNE

(30) Priority: 19.04.2024 TW 113114651
(43) Date of publication of application: 22.10.2025
(73) Proprietor: Golden Phoenix Fiberwebs, Inc., Tainan City 730 (TW)
(72) Inventor: Cheng, Kenneth, Taipei City (TW)
(74) Representative: Stevens Hewlett & Perkins

(56) References cited:
- GB-A- 792 355
- GB-A- 971 430
- JP-A- S5 135 792
- US-A1- 2024 075 704

## Description

### CROSS-REFERENCE TO RELATED APPLICATION

This application claims the priority of Taiwanese patent application No. 113114651, filed on April 19, 2024.

### BACKGROUND OF THE INVENTION

### 1. Field of the Invention

The present invention relates to a non-woven fabric with elasticity in warp direction and a manufacturing method thereof, specially a non-woven fabric with elasticity in warp direction in which wavy folds are firstly formed, and the orientation of fibers of non-woven fabric are changed and the non-woven fabric is imparted with elasticity through heat softening, stretching in weft direction, and cooling and setting, and then the wavy folds are straightened, and a manufacturing method thereof.

### 2. The Prior Arts

General sanitary products, such as masks, disposable clothing, infant diapers or adult diapers, or sport protective bandages, medical bandages, etc., are usually provided in disposable forms when considering hygiene and using safety to avoid contamination of germs or harmful substances. Because such products will be in contact with the skin for a period of time, there are stricter requirements on breathability to prevent discomfort, skin allergies, itching, and even rashes caused by hot or humid conditions.

Since non-woven fabrics made of plastic materials have the advantages of easy manufacturing, processing, good chemical resistance, durability and low cost, they have been widely used in many sanitary products. However, non-woven fabrics have poor extensibility, insufficient comfort and cladding properties, which may cause inconvenience in wearable applications such as diapers. Therefore, composite non-woven fabrics with improved extensibility have been developed in the industry, which can be referred as to elastic composite non-woven fabrics.

In an existing manufacturing process of elastic composite non-woven fabrics, a common method is to pre-stretch a piece of elastic material as a middle layer, and then use two pieces of general non-woven fabrics without elasticity as upper and lower layers, respectively, perform bonding in a sandwich manner, and stop applying external force for stretching after bonding to form wavy folds on upper and lower surfaces of the elastic composite non-woven fabric; the other common method is to use a piece of elastic material as a middle layer without stretching, and then use two pieces of general non-woven fabrics without elasticity as upper and lower layers, respectively, perform bonding in a sandwich manner to form a three-layer structure in a flat shape, after bonding, the material surface of the general non-woven fabric is damaged, such as activated, to make the general non-woven fabric slightly extensible.

In another existing method such as patent publication US 2024/075704 Al, a composite nonwoven fabric is produced to achieve high extensibility and tensile strength. In this document, two ordinary inelastic non-woven fabrics are subjected to heat contraction to be imparted initial extensibility, and then formed with wavy pleats using pairs of grooved rolls. These pre-shrunk elastic nonwoven layers are subsequently bonded to the top and bottom sides of a middle layer of elastic material. This specific structure results in a two-stage extensibility, where the first stage involves stretching the composite nonwoven fabric from a wavy state back to a flat state of the elastic nonwoven layers, and the second stage involves in stretching the composite nonwoven fabric to its tensile limit.

However, in the existing manufacturing process of multiple layered elastic nonwoven fabric composite, including the method disclosed in US 2024/075704 Al, in addition that there are more manufacturing steps, the bonding also makes the non-woven product thicker, causing poor comfort to user, and increasing the space and cost required for storage and transportation. Also, peeling phenomenon of the product may be occurred due to incomplete bonding. Moreover, if the bonding is performed by an adhesive, the peeling phenomenon may easily occur due to non-uniform distribution of the adhesive.

Another existing technique is to use elastomers as raw materials to manufacture a single-layered elastic non-woven fabric through processes for non-woven fabric such as melt-blowing or spun-bonding, however, the cost thereof is high. Therefore, an object of the present invention is to develop an elastic non-woven fabric, which imparts elasticity to a single-layered non-woven fabric only by the thermoplastic property of synthesized fibers, thereby having the advantage of significantly reduced costs.

Among the existing non-woven fabric manufacturing process, in addition to spun-bonding process, there are also other processes such as spunlace, needle-punching, and melt-blowing. The spun-bonding process refers a method in which raw materials are melted through an extrusion equipment and extruded from a nozzle, stretched and cooled via an air duct to form ultra-fine fibers, and then blown toward a collecting net and accumulate into a network structure, and the long fibers with a disordered network structure pass through a heated hot roller, thereby performing hot-pressing and bonding for the fiber layer.

Due to the thermoplastic property of the plastic non-woven fabrics (soft when being heated and hard after being cooled) and a non-oriented distribution property of the fiber tissue of general non-woven fabrics (as shown in FIG. 1a, the fiber tissue 11 of the non-woven fabric is randomly oriented), hot airflow can be used to penetrate the fiber tissue to heat the fibers to the corresponding softening temperature, and while heating and softening, the distributed fibers are mechanically stretched continuously in the weft direction to change the orientation of the fiber tissue (the non-woven fabric in FIG. 1a is stretched in the weft direction such that the fiber tissue 11 is oriented in the weft direction to a status shown in FIG. 1b, while the non-woven fabric is necked in the warp direction).

Since the orientation of the fibers in the fiber tissue 11 of the non-woven fabric contributes to providing elasticity, after the elastic non-woven fabric that has been softened by heating and stretched in the weft direction is cooled, its fiber tissue forms a state of a telescopic robotic arm as shown in FIG. 1b, wherein when a stretching force in the warp direction is applied, the fiber tissue 11 oriented in the weft direction of the non-woven fabric (as shown in FIG. 1b) can be stretched along the warp direction back to a state where the fiber orientation has not been altered (as shown in FIG. 1a), thereby providing extensibility in the warp direction; moreover, after stop applying the stretching force in the warp direction, the fiber tissue 11 of the elastic non-woven fabric will restore to the state being oriented in the weft direction (as shown in FIG. 1b), thereby providing a restoring ability in the warp direction; that is, such elastic non-woven fabric has a stretching and restoring ability in the warp direction.

On the other hand, FIG. 2a and FIG. 2b respectively show the microscopic images of general spunlace non-woven fabric before and after being stretched in the weft direction, in which it can be also observed that the fiber tissue of the non-woven fabric is oriented in the weft direction after being stretched.

In addition, a necking deformation of the non-woven fabrics will occur (see the necking area N in FIG. 3) after mechanical stretching in the weft direction, and the area in the warp direction of the non-woven fabric material will be reduced due to the Poisson's ratio. Therefore, by overfeeding the non-woven fabric along the warp direction in advance (that is, the fabric feeding speed is greater than the running speed of the needle clips), the non-woven fabric can form a wavy state, so as to reduce the tension in the warp direction of the fabric, thereby compensating the necking phenomenon mentioned above, and preventing the non-woven fabric from becoming too thin due to the necking phenomenon after stretching, which facilitates the broadening in the weft direction.

However, conventional overfeeding simply based on speed difference will cause uneven wavy folds of the non-woven fabrics, which will lead to a problem of uneven fabric surface after broadening in the weft direction. Therefore, there is a need for an improved manufacturing method of an elastic non-woven fabric.

Further, patent publication GB 792355 A discloses a modification in conventional tentering machines, in which a woven or knitted fabric is supplied at overfeed to a tenter machine with two pin conveyors. Specifically, the fabric is initially supplied through a nip between a pair of feed rolls and then pushed by a brush onto the pins of the conveyors.

Patent publication GB 971430 A discloses another modification in conventional tentering machines, in which the fabric web is pleated as it is supplied at overfeed to a nip defined between a roll and an endless corrugated band, and then pushed by a brush onto the conveyor pins. Specifically, the fiber web is pressed into the troughs in the corrugated band by an impressing roller encircled by a ring of foam rubber or foam plastic to be undulated, and then brushed onto the conveyor pins.

Patent publication JP S5135792 A discloses yet another modification in conventional tentering machines, in which a flexible endless belt with pins that forms a curved surface is used. By utilizing the geometric difference between the expanded pin spacing at the curved portion and the retracted spacing at the flat portion, uniform pleats are formed on the fabric.

Despite some prior art documents describing that these fabrics may then be subjected to the conventional tentering process, such as drying, thermal setting, stretching and cooling, the tenter devices therein are set up for conventional tentering of woven or knitted fabrics. That is, none of those documents suggest an improvement in tentering process of nonwoven fabric.

### SUMMARY OF THE INVENTION

In view of the problems encountered in the prior art, the present invention is to provide a manufacturing method of a non-woven fabric with elasticity in warp direction, in which by pre-forming regular wavy folds on the non-woven fabric and using an air suction device, the reduced area or reduced thickness of the non-woven fabric caused by necking during subsequent stretching can be compensated, thereby improving the unevenness by conventional overfeeding; and a single-layered elastic non-woven fabric manufactured according to the above method, which has strong resilience in the warp direction and has a flat surface. Therefore, it can be directly used in products without being bonded to another elastic base material, thereby greatly improving production rate, improving comfort to user, and reducing the space and cost required for storage and transportation.

In order to solve the above problems, the present invention provides a manufacturing method of an elastic non-woven fabric, comprising:
a feeding step, using at least two feeding wheel sets to feed a non-woven fabric, wherein the feeding wheel sets are respectively located at both sides in a weft direction of the non-woven fabric, and each feeding wheel set includes a speed differential gear and a suction gear that engage with each other, wherein each speed differential gear is provided with a plurality of first teeth portions and a plurality of first groove portions alternately arranged along an outer circumferential surface of the speed differential gear, and each suction gear is provided with a hollow groove at a center in the weft direction on an outer surface thereof, and each suction gear is provided with a plurality of second teeth portions, a plurality of second groove portions and a plurality of suction holes at both sides in the weft direction of the hollow groove, respectively, wherein the second groove portions and the second teeth portions are alternately arranged along both sides in the weft direction of an outer circumferential surface of the suction gears, respectively, and the suction holes are provided at least on the second groove portions, wherein the speed differential gears feed both sides in the weft direction of the non-woven fabric into a location between the speed differential gears and the suction gears respectively along a warp direction;
a wave forming step, rotating the speed differential gears and the suction gears with engaging with each other in a manner that the first teeth portions are inserted into the second groove portions and the second teeth portions are inserted into the first groove portions, such that both sides in the weft direction of the non-woven fabric respectively enter a location between the first teeth portions and the second groove portions and a location between the first groove portions and the second teeth portions, thereby forming regular wavy folds on the non-woven fabric along the warp direction;
a fixing step, using the suction gears and at least two pin chains in a form of conveyor belt to fix the wavy folds of the non-woven fabric, wherein the pin chains are respectively located on both sides in the weft direction of the non-woven fabric, and the feeding wheel sets are respectively arranged above the pin chains, and a plurality of pins are provided on each pin chain, wherein a suction force is provided through the suction holes to make both sides in the weft direction of the non-woven fabric closely fit outer surfaces of the second teeth portions and the second groove portions, respectively, and the pin chains run in the form of conveyor belt while the suction gears rotate, making the pins puncture the non-woven fabric and enter the hollow grooves, respectively, to fix the wavy folds of the non-woven fabric, and the suction gears stop providing the suction force after the pins puncture the fed non-woven fabric, such that the non-woven fabric can be smoothly transferred from the suction gears to the pin chains;
a press-flattening step, press-flattening the wavy folds of the non-woven fabric through at least two brush wheels, wherein the brush wheels are respectively disposed above the pin chains at downstream in the warp direction of the feeding wheel sets, and the brush wheels rotate while the pin chains run in the form of conveyor belt, so as to press-flatten the wavy folds of the non-woven fabric on the pin chains;
a preheating step, using the pin chains to transport the non-woven fabric along the warp direction with maintaining a fixed distance in the weft direction of the pin chains, meanwhile, using a heating device to heat the non-woven fabric to soften it;
a broadening step, under proceeding the heating of the heating device, using the pin chains to transport the softened non-woven fabric along the warp direction with the distance in the weft direction of the pin chains gradually increased to stretch the non-woven fabric in the weft direction, such that a necking compensation effect of the non-woven fabric occurs along the warp direction to straighten the wavy folds that extend along the warp direction and are press-flattened, thereby making a fiber tissue of the non-woven fabric be oriented along the weft direction, such that the non-woven fabric is in a flat shape and has a stretching and restoring ability along the warp direction;
a stabilizing step, under proceeding the heating of the heating device, using the pin chains to transport the softened and stretched non-woven fabric along the warp direction with maintaining the increased distance in the weft direction for stabilizing the non-woven fabric; and
a cooling step, cooling the stabilized non-woven fabric to set it, thereby forming a non-woven fabric with elasticity in the warp direction;
wherein in the feeding step, the speed differential gears feed the non-woven fabric into the location between the speed differential gears and the suction gears along the warp direction at a speed higher than a conveying speed of the pin chains.

In an embodiment of the present invention, the suction holes are further provided on the second teeth portions.

In an embodiment of the present invention, the heating temperature in the preheating step, the broadening step and the stabilizing step is 120 to 180°C, preferably 130 to 150°C.

In an embodiment of the present invention, in the broadening step, a broadening ratio of the non-woven fabric in the weft direction is between 15 and 100%.

In an embodiment of the present invention, in the fixing step, respective pins on the pin chains are aligned with a peak and/or a trough of the wavy folds, respectively.

In an embodiment of the present invention, a ratio of a spacing between the first teeth portions, a spacing between the second teeth portions, and a spacing between the pins is 1:1:1 or 1:1:0.5.

In an embodiment of the present invention, the non-woven fabric is made by spun-bonding, spunlace, thermal-bonding, melt-blowing, or needle-punching.

In an embodiment of the present invention, the non-woven fabric is made of a material selected from a group consisting of PP, PE, PET, PP/PE, PP/PET, or a combination thereof.

In order to solve the above problems, the present invention also provides a non-woven fabric with elasticity in warp direction, wherein the non-woven fabric with elasticity in warp direction has a flat surface and has a fiber tissue substantially oriented in the weft direction, such that the non-woven fabric with elasticity in warp direction has a stretching and restoring ability along the warp direction.

In an embodiment of the present invention, the non-woven fabric with elasticity in warp direction has an elongation in the warp direction between 50 and 350%.

The effects of the present invention are that: first, by feeding the non-woven fabric through the speed differential gears and the suction gears that engage with each other, regular wavy folds can be formed on the non-woven fabric, which is beneficial to ensure the surface flatness of the final elastic non-woven fabric; second, by providing a suction force through the suction gears to make the non-woven fabric closely fit outer surfaces of the teeth portions and groove portions of the suction gears, the non-woven fabric with the wavy folds can be transferred to the subsequent process with maintained shape, which is beneficial to improve the uniformity of the final fabric surface; third, by disposing a hollow groove at a center on the outer surfaces of the suction gears, a space for accommodating the pins on the pin chains after the pins puncture the non-woven fabric can be provided; fourth, by slightly stretching in the weft direction under heating to change the fiber orientation and subsequent cooling and setting, the non-woven fabric can have better elasticity in the warp direction than the prior art; fifth, by pre-forming regular wavy folds, the reduced area or reduced thickness of the non-woven fabric caused by necking during subsequent stretching can be compensated; sixth, by making the single-layerd non-woven fabric have excellent elasticity after processing, additional bonding materials or bonding steps can be omitted, thereby reducing the manufacturing costs and making the product thinner to improve comfort to user, and reducing the space and cost required for storage and transportation.

The effects of the present invention are not limited to the effects described above, and a person skilled in the art can clearly understand other effects not mentioned from the description of the claims.

### BRIEF DESCRIPTION OF THE DRAWINGS

FIG. 1a and FIG.1b respectively show images of general spunbond non-woven fabrics before and after being stretched in the weft direction (photographed by a hand-held low-noise and high-definition digital microscope);
FIG. 2a and FIG.2b respectively show images of general spunlace non-woven fabrics before and after being stretched in the weft direction (photographed by a hand-held low-noise and high-definition digital microscope);
FIG. 3 shows a perspective view of a manufacturing equipment for a non-woven fabric with elasticity in warp direction of the present invention;
FIG. 4 shows a schematic diagram showing pins entering a hollow groove in the manufacturing equipment of the present invention, in which the non-woven fabric is not shown;
FIG. 5a shows a schematic diagram of wavy folds, which are formed only by a differential wheel with a flat surface, being press-flattened by a brush wheel in a setting machine in the prior art;
FIG. 5b shows the differential wheel of the setting machine in the prior art;
FIG. 6a shows a schematic diagram of the uneven wavy folds formed by the setting machine in the prior art;
FIG. 6b shows a schematic diagram of the uneven wavy folds formed by the setting machine in the prior art after being press-flattened by the brush wheel;
FIG. 7 shows a schematic diagram of the wavy folds, which are formed by feeding wheel sets including speed differential gears and suction gears in forms of gear, being press-flattened by a brush wheel in the manufacturing equipment of the present invention;
FIG. 8a shows a schematic diagram of the uniform wavy folds formed by the manufacturing equipment of the present invention;
FIG. 8b shows a schematic diagram of the uniform wavy folds formed by the manufacturing equipment of the present invention after being press-flattened by the brush wheel;
FIG. 9a shows a photo of a final fabric manufactured by the setting machine in the prior art;
FIG. 9b shows a photo of a final non-woven fabric manufactured by the manufacturing equipment of the present invention;
FIG. 10 shows a flow chart of a manufacturing method of the non-woven fabric with elasticity in warp direction of the present invention;
FIG. 11 shows a schematic diagram of an appearance of the non-woven fabric with elasticity in warp direction of the present invention; and
FIG. 12 shows a partial enlarged view of a region a of FIG. 11.

### DETAILED DESCRIPTION OF THE PREFERRED EMBODIMENT

The advantages and features and the implementing method thereof of the present invention will be more clearly understood from the embodiments described below with reference to the accompanying drawings. However, the present invention is not limited to the following embodiments, but may be implemented in various different forms.

The technical features of any aspect of the present invention can be combined with those of other aspects of the present invention without contradiction.

Herein, "MD (Machine direction)" refers to a direction parallel to the direction of the manufacturing equipment transporting the non-woven fabrics, also called as the warp direction; and "TD (Transverse direction)" refers to a direction vertical to the direction of the manufacturing equipment transporting the non-woven fabrics.

Herein, "Broaden ratio" refers to a ratio of the final stretching amount of a material (such as a raw material of non-woven fabric) relative to its original width to an original width of the material during a broadening stage.

Herein, "Elonation" refers to a ratio of a maximum elongation amount of a material (such as a non-woven fabric with elasticity in warp direction) relative to its natural width to a natural width of the material.

Referring to FIG. 3, the present invention provides a manufacturing equipment of a non-woven fabric with elasticity in warp direction, comprising: a heating device 60, a pin chain 40 in the form of conveyor belt, feeding wheel sets F, and a brush wheel 50.

The heating device 60 has an inlet 61, an internal space 62 and an outlet 63 in sequence along the warp direction, wherein the internal space 62 is divided into a preheating section 62a adjacent to the inlet 61, a broadening section 62b in the middle, and a stabilizing section 62c adjacent to the outlet 63 in the warp direction.

In the present invention, the non-woven fabric can be softened by heat for processing and shaping by the heating device 60, such as an oven, but not limited thereto. The internal space 62 of the heating device 60 is the space that is actually heated, and the inlet 61 and the outlet 63 of the heating device 60 can be designed to be heated or not heated depending on demand.

Since non-woven fabrics 10 with different components have different softening points, the heating temperature for the heating device 60 can be 120 to 180°C, preferably 130 to 150°C.

The number of the pin chains 40 is at least two, and the two are located at both sides of the heating device 60 in the weft direction, respectively, and extends from the inlet 61, through the preheating section 62a, the broadening section 62b and the stabilizing section 62c, to the outlet 63 of the heating device 60 in sequence along the warp direction. Each pin chain 40 is provided with a plurality of pins 41.

Referring to FIG. 3, the number of the feeding wheel sets F is at least two, and the two are respectively disposed above the pin chains 40 at both sides of the inlet 63 of the heating device 60.

Each feeding wheel set F includes speed differential gears 20 and suction gears 30 that engage with each other.

Each speed differential gear 20 is provided with a plurality of first teeth portions 21 and a plurality of first groove portions 22, which are alternately arranged along an outer circumferential surface of the speed differential gear 20.

Referring to FIG. 4, each suction gear 30 is provided with a hollow groove 34 at a center in the weft direction on an outer surface thereof; and each suction gear 30 is provided with a plurality of second teeth portions 31, a plurality of second groove portions 32 and a plurality of suction holes 33 at both sides in the weft direction of the hollow groove 34, respectively, wherein the second groove portions 32 and the second teeth portions 31 are alternately arranged along both sides of the weft direction of the outer circumferential surface of the suction gears 30, respectively, and the suction holes 33 are provided at least on the second groove portions 32.

Referring to FIG. 3, the number of the brush wheels 50 is at least two, and the two are respectively disposed above each pin chain 40 at downstream in the warp direction of each feeding wheel set F.

In the manufacturing equipment of the present invention, the pin chains 40, the feeding wheel sets F, and the brush wheels 50 are preferably symmetrically arranged relative to each other at both sides in the weft direction of the heating device 60, which is beneficial to the smooth transportation of the non-woven fabric and avoids pulling and drag or unevenness of the non-woven fabric during the processing.

In addition, although in the specification, the configuration including two pin chains 40, two feeding wheel sets F, and two brush wheels 50 are taken as an example for describing, a person skilled in the art can understand that additional pin chain(s) 40, feeding wheel set(s) F and brush wheel(s) 50 can be appropriately added between the above components, depending on the trade-off between the equipment cost and the processing precision according to product requirements.

In the present invention, a general non-woven fabric 10 is processed by the manufacturing equipment of the non-woven fabric with elasticity in warp direction, thereby the orientation of the fibers is changed after heat-softening, stretching in the weft direction, and cooling and setting, so as to be oriented in the weft direction, thereby imparting the non-woven fabric an elasticity in the warp direction.

Preferably, the non-woven fabric 10 includes, but is not limited to those made by spun-bonding, spunlace, thermal-bonding, melt-blowing or needle-punching.

In order to meet the heat-softening and cool-setting characteristics required in the manufacturing process, the non-woven fabric 10 used in the present invention is made of thermoplastic materials, such as polypropylene (PP), polyethylene (PE), polyethylene terephthalate (PET), two-component PP/PE, two-component PP/PET, or a combination thereof, but not limited thereto.

The operation manner of the manufacturing equipment of the non-woven fabric with elasticity in warp direction of the present invention is explained below.

First, the speed differential gears 20 feeds both sides in the weft direction of the non-woven fabric 10 into each set of the speed differential gears 20 and the suction gears 30 along the warp direction respectively at a conveying speed higher than that of the pin chains 40 (that is, in an overfeeding manner), wherein each set of the speed differential gears 20 and the suction gears 30 engage and rotate with each other in a manner that the first teeth portions 21 are inserted into the second groove portions 32 and the second teeth portions 31 are inserted into the first groove portions 22, such that both sides in the weft direction of the non-woven fabric 10 respectively enter a location between the first teeth portions 21 and the second groove portions 32 and a location between the first groove portions 22 and the second teeth portions 32, thereby forming regular wavy folds on the non-woven fabric 10 along the warp direction.

Then, the suction gears 30 provides a suction force through the suction holes 33 at least disposed on the second groove portions 32, such that both sides in the weft direction of the fed non-woven fabric 10 closely fit outer surfaces of the second teeth portions 31 and the second groove portions 32, respectively.

Preferably, in order to enhance the effect of making the non-woven fabric 10 closely fit the outer surfaces of the second teeth portions 31 and the second groove portions 32 of the suction gears 30, the suction holes 33 may be further disposed on the second teeth portions 31.

Subsequently, the hollow groove 34 of the suction gears 30 is configured to allowed the pins 41 of the pin chains 40 to puncture the fed non-woven fabric 10 and enter the hollow groove 34 when the pin chains 40 run in the form of conveyor belt while the suction gears 30 rotate, for fixing the wavy folds of the fed non-woven fabric 10.

Moreover, the suction gears 30 stop providing the suction force after the pins 41 puncture the fed non-woven fabric 10, such that the non-woven fabric 10 can be smoothly transferred from the suction gears 30 to the pin chains 40.

Then, the brush wheel 50 rotates while the pin chains 40 run in the form of conveyor belt, so as to press-flatten the wavy folds of the non-woven fabric 10 on the pin chains 40. In order to process smoothly, the brush wheel 50 is configured to has a height that allows the wavy folds of the non-woven fabric 10 fixed on the pin chains 40 to be press-flattened when the brush wheel rotates above the pin chains 40.

In addition, in order to press-flatten the wavy folds of the non-woven fabric 10 before stretching and broadening (to be described later) the non-woven fabric 10 , the brush wheel 50 can be specifically arranged within the range from downstream in the warp direction of the feeding wheel sets F to the softening section 62a of the heating device 60.

In the prior art, since the fabric will shrink after being dyed with high-temperature water, a setting machine will be used to broaden the fabric during the high-temperature drying process to compensate the shrinkage and to set the fabric, so as to make the width of the fabric consistent, and to stabilize the straight arrangement of the warp and weft yarns, and also to adjust the feel of the fabric; in addition, the arrangement of the warp and weft yarns can be more finely adjusted during broadening by using the overfeeding technology.

The above prior art is applied to the fabrics with the arrangement of warp and weft yarns; and in the broadening and setting process of the fabrics using the overfeeding technology, the factors such as the denier value (tensile strength), the arrangement of warp and weft yarns (tensile strength of tissue arrangement) and the thread count (tensile strength of density) of the fabrics and their adjustable ranges have been fixed and cannot be adjusted by a larger extent.

During the development of the present invention, when the setting machine and overfeeding technology in the above prior art are applied to the non-woven fabrics, it is found that: unlike fabrics with the arrangement of warp and weft yarns, the fibers of the non-woven fabrics have disoriented arrangement, in which the effect of broadening and setting, as well as necking by overfeeding can be increased. However, the overfeeding technology applied in the above prior art will affect the uniformity of the non-woven fabrics due to lacking the design of gears and suction devices (as shown in FIG. 9a).

In the present invention, through the improved design of the speed differential gears 20 and the suction gears 30, regular wavy folds can be formed on the non-woven fabric 10 and then transferred to the pin chains with maintained shape, which avoids the problem of uneven wavy folds caused by fabric overfeeding simply based on speed difference, and a problem of uneven thickness of the final fabric after broadening in the weft direction in the broadening and setting process of the prior art.

As shown in FIGs. 5a to 5b, in the fabric setting machine of the prior art, there is only a configuration of a differential wheel 20' and a brush wheel 50', without the suction gear. Wherein, a belt wheel B' and the differential wheel 20' overfeed the non-woven fabric 10' into a location between the differential wheel 20' and the brush wheel 50', thereby generating an overfeeding difference based on a feeding speed of belt wheel B' and the differential wheel 20' being greater than a conveying speed of pin chains 40', using the belt wheel B' and the differential wheel 20' to clamp the non-woven fabric 10' to cause squeezing by speed difference, so as to form wavy folds, and then using the brush wheel 50' to press the non-woven fabric 10' into the pin chains 40'.

Preferably, as shown in FIG. 5b, the differential wheel 20' has a friction surface 20a' at one side of the circumferential surface thereof, and a brush 20b' at the other side, and the brush 20b' on the differential wheel 20' can also used to press the non-woven fabric 10' into the pin chains 40'.

However, since the differential wheel 20' of the prior art has a flat surface without teeth portion, it can only provide friction between it and the non-woven fabric 10' through a friction surface thereof (for example, made of rubber material).

Therefore, this configuration will cause uneven wavy folds of the non-woven fabric, which will lead to a problem of uneven fabric surface after broadening in the weft direction. Specifically, while the differential wheel 20' rotates, the pins 41' on the pin chains 40' puncture and fix the uneven wavy folds of the non-woven fabric 10' (as shown in FIG. 6a), and after the brush wheel 50' further press-flattens the wavy folds, only the non-woven fabric 10' having uneven wavy folds being press-flattened can be obtained (as shown in FIG. 6b). Therefore, uniform broadening cannot be achieved in the subsequent process, thereby leading to a problem of unevenness in the final fabric surface.

Referring to FIGs. 7 to 8b, the manufacturing equipment of the present invention is different from the prior art in that: in the present invention, the flat differential wheel 20' of the prior art is replaced by the speed differential gear 20 in form of gear, and the suction gear 30 is further provided.

As the speed differential gears 20 and the suction gears 30 mesh with each other and rotate, the non-woven fabric 10 will enter a location between teeth portions and groove portions of the speed differential gears 20 and the suction gears 30, thereby forming regular wavy folds on the non-woven fabric 10 along the warp direction.

Thereafter, since the suction holes 33 are disposed on the surface of the suction gears 30, by providing a suction force through the suction holes 33 to make the non-woven fabric 10 closely fit outer surfaces of the second teeth portions 31 and the second groove portions 32 of the suction gears 30, thereby temporarily fixing the wavy folds of the non-woven fabric 10 through suction force, the wavy folds of the non-woven fabric 10 can be transferred to the subsequent process with maintained shape, which facilitates the subsequent fixing through the pin chains 40, so as to avoid the non-woven fabric 10 from shifting during the subsequent process, thereby improving the uniformity of the final non-woven fabric surface.

After that, as the suction gears 30 rotate, the non-woven fabric 10 having wavy folds move to the upper location the pin chains 40, and as the pin chains 40 run in the form of conveyor belt, the pins 41 on the pin chains 40 puncture and fix the regular wavy folds of the non-woven fabric 10 (as shown in FIG. 8a); subsequently, after the brush wheel 50 further press-flattens the wavy folds, the non-woven fabric 10 having regular wavy folds being press-flattened can be obtained (as shown in FIG. 8b). Therefore, uniform broadening can be achieved in the subsequent process, thereby a non-woven fabric with elasticity in warp direction having an uniform fabric surface can be manufactured.

FIG. 9a and FIG. 9b show photos of the final fabric manufactured by the manufacturing equipment of the prior art and the final non-woven fabric manufactured by the manufacturing equipment of the present invention, respectively. Wherein, when the differential wheel 20' of the prior art is used, the final fabric has uneven folds, and when the speed differential gears 20 and the suction gears 30 of the present invention are used, the final non-woven fabric has flat surface appearance.

Preferably, the spacing or arranging density between the pins 41 of the pin chains 40 can be adjusted to increase the degree of fixing of the pin chains 40 to the non-woven fabric 10.

Preferably, multiple sets of pin chains 40 can be provided, and the number of teeth portions and the distance between pin chains can be adjusted depending on demand in elastic extension.

Preferably, the speed differential gears 20 and the suction gears 30 can be designed to have same diameter and same number of teeth portions, thus a rotating speed ratio of the speed differential gears 20 to the suction gears 30 can be 1:1.

Preferably, compared with the manufacturing equipment of the non-woven fabric with elasticity in warp direction of the prior art, the number of teeth portions of the speed differential gears 20 and the suction gears 30 can be increased or decreased and replaced by modules, and the number and height of the teeth portions and the groove portions can also designed correspondingly to the pin chains 40.

Preferably, the manufacturing equipment of the present invention can be designed such that respective pins 41 are respectively aligned with a peak and/or a trough of the wavy folds of the non-woven fabric 10 (as shown in FIG. 8a), therefore, the wavy folds can be better fixed in subsequent processes.

Preferably, a ratio of a spacing between the first teeth portions 21, a spacing between the second teeth portions 31, and a spacing between the pins 41 can be designed to be 1:1:1, such that respective pins 41 can be respectively aligned with each peak or trough of the wavy folds of the non-woven fabric 10.

Alternatively, in a more preferred embodiment, a ratio of a spacing between the first teeth portions 21, a spacing between the second teeth portions 31, and a spacing between the pins 41 can be designed to be 1:1:0.5, such that respective pins 41 can be respectively aligned with each peak and trough of the wavy folds of the non-woven fabric 10 (as shown in FIG. 8a).

Preferably, in the manufacturing equipment of the present invention, by adjusting the height and width of the first teeth portions 21 and the second teeth portions 31, the width of the first groove portions 22 and the second groove portions 32, and the distance between the speed differential gears 20 and the suction gears 30, the height or width of the wavy folds of the non-woven fabric 10 can be adjusted, that is, the shape of the wavy folds of the non-woven fabric 10 can be changed.

The thickness, elasticity in warp direction and uniformity of the final non-woven fabric with elasticity in warp direction can be adjusted by changing the shape of the wavy folds of the non-woven fabric.

There is an corresponding relationship between the height or width of the wavy folds, the distance between the two types of wheels, and the uniformity of the fabric, for example, when the number of gears and the distance of the gears are fixed, if the broadening amount in the weft direction is large, the distance between the two types of wheels will be short (the height of the wavy folds is large), there are enough amount of fibers to be stretched toward both sides, the fabric is slightly thicker, the necking amount is large, and the elasticity in the warp direction is good; if the broadening amount in the weft direction is small, the distance between the two types of wheels is long (the height of the wavy folds is small, the necking amount is small, and the elasticity in the warp direction is poor. The elasticity in the warp direction can be controlled and adjusted according to needs, and the weight of the fabric can be maintained uniform.

On the other hand, if the broadening amount in the weft direction is large, the distance between the two types of wheels will be long (the height of the wavy folds is small), the necking amount is large, and the amount of fibers is insufficient due to the less number of folds, there will be a problem of uneven surface and uneven weight of the fabric; if the broadening amount in the weft direction is small, the distance between the two types of wheels will be short (the height of the wavy folds is large), the fabric will become thicker and has reduced elasticity.

Specifically, under the same broadening ratio, the height and uniformity of the wavy folds will affect the flatness of the fabric (i.e., causing uneven weight per unit area of the fabric), and in the process of broadening in the weft direction, stretching, and necking under appropriate temperatures, the fibers with wavy folds having large height and even arrangement are easier to be expanded evenly; however, when the height of the wavy folds is small and the wavy folds are unevenly arranged, the fibers at thinner portions of the fabric will be stretched first and unevenly, such that the thickness of the fabric becomes thinner, moreover, when the wavy folds are arranged densely in some portions and loosely in the other portions, uneven continuously necking in the warp direction will occurred.

The present invention is advantageous compared with the prior art in that: the height and arrangement uniformity of the wavy folds can be adjusted; a stable continuously necking in the warp direction of the non-woven fabric can be generated through precisely control of the process conditions, such that a continuous shrinkage ratio in the warp direction of each portion of the fabric can be consistent (continuous elasticity); and controlling the elastic stretching and restoring effect of the non-woven fabric and achieving uniform weight per unit area of the fabric.

Subsequently, the pin chains 40 transports the non-woven fabric 10 with the press-flattened wavy folds to the internal space 62 of the heating device 60 along the warp direction from the inlet 61 of the heating device 60.

After that, in the preheating section 62a of the heating device 60, under the condition that the pin chains 40 respectively fixing both sides of the non-woven fabric 10 maintain at a fixed distance in the weft direction, that is, without changing the width of the non-woven fabric 10, the pin chains 40 transport the non-woven fabric 10 into the broadening section 62b along the warp direction; at the same time, the heating device 60 heats the non-woven fabric 10 to soften it for subsequent processing and shaping.

Subsequently, in the broadening section 62b of the heating device 60, the heating device 60 proceeds to heat the non-woven fabric 10 to maintain it at the softening temperature; while under the condition that the distance in the weft direction of the pin chains 40 respectively fixing both sides of the weft direction of the non-woven fabric 10 gradually increase, the pin chains 40 proceed to transport the softened non-woven fabric 10 along the warp direction, so as to stretch the non-woven fabric 10 along the weft direction by the gradually increased distance in the weft direction of the pin chains 40, thereby increasing the width in the weft direction of the non-woven fabric 10.

Preferably, a broadening ratio of the non-woven fabric 10 in the weft direction in the broadening section 62b can be, for example, between 15 and 100% (that is, the non-woven fabric 10 is finally stretched to a width in the weft direction 1.15 to 2 times of its original width in the weft direction in the broadening section 62b).

For example, the width in the weft direction of the non-woven fabric is 100 cm, after broadening in the weft direction and stretching, the width in the weft direction becomes 115 cm, thus the broadening ratio in the weft direction is 115%. For another example, the width in the weft direction of the non-woven fabric is 100 cm, after broadening in the weft direction and stretching, the width in the weft direction becomes 200 cm, thus the broadening ratio in the weft direction is 200%.

In addition, a broadening ratio in the weft direction of commercially available setting machines can be up to 450%, for example.

During the stretching in the weft direction, the fibers of the non-woven fabric 10 are mechanically continuously stretched in the weft direction by the spacing gradually increased in the weft direction of the pin chains 40, which changes the orientation of the fiber tissue, thereby making the fiber tissue of the non-woven fabric 10 be oriented along the weft direction, so as to impart the non-woven fabric 10 a stretching and restoring ability along the warp direction; at the same time, due to the stretching in the weft direction, a necking compensation effect of the non-woven fabric 10 occurs along the warp direction due to the Poisson's ratio, thereby straightening the wavy folds that extend along the warp direction and are press-flattened, such that the fabric is in a flat shape.

Next, in the stabilizing section 62c of the heating device 60, the heating device 60 proceeds to heat the non-woven fabric 10 to maintain it at the softening temperature; while under the condition that the pin chains 40 respectively fixing both sides of the weft direction of the non-woven fabric 10 maintain at the increased distance in the weft direction, that is, the non-woven fabric 10 maintains at the broadened width, the pin chains 40 transport the softened and stretched non-woven fabric 10 along the warp direction, such that the non-woven fabric 10 is kept in a softened and broadened state for a period of time, thereby stabilizing the stretched and broadened non-woven fabric 10.

Finally, the pin chains 40 fixing both sides of the weft direction of the non-woven fabric 10 transport the stabilized non-woven fabric 10 out of the heating device 60 from the outlet 63, thereby cooling the stabilized non-woven fabric to set it, that is, to set it in a state of being stretched, broadened, and having elasticity in the warp direction, thereby forming the non-woven fabric with elasticity in warp direction of the present invention.

After cooling and setting, the fiber tissue of the non-woven fabric 10 is oriented along the weft direction and forms a state of a telescopic robotic arm (as shown in FIG. 1b), when a stretching force in the warp direction is applied, the fiber tissue oriented in the weft direction of the non-woven fabric 10 can be stretched along the warp direction back to a state where the fiber orientation has not been altered, therefore, the non-woven fabric 10 has extensibility in the warp direction; moreover, after stopping applying the stretching force in the warp direction, the elastic non-woven fabric will restore to the state being oriented in the weft direction, therefore, the non-woven fabric 10 has a restoring ability in the warp direction. Therefore, the orientation in the weft direction formed by stretching and broadening along the weft direction imparts the non-woven fabric with elasticity in warp direction of the present invention a high stretching and restoring characteristic that is superior to the elastic non-woven fabric of the prior art.

Referring to FIG. 10, which shows a flow chart of a manufacturing method of the non-woven fabric with elasticity in warp direction of the present invention. The manufacturing method of the elastic non-woven fabric of the present invention comprises: a feeding step S10, a wave forming step S20, a fixing step S30, a press-flattening step S40, a preheating step S50, a broadening step S60, a stabilizing step S70, and a cooling step S80.

The elements used in the following steps, such as the heating device, the pin chain, the feed wheel set and the brush wheel, can be the elements mentioned above, such as the heating device 60, the pin chain 40, the feed wheel set F and the brush wheel 50. Therefore, the features and details of these elements will not be described again.

In the feeding step S10, at least two feeding wheel sets are used to feed a non-woven fabric, wherein speed differential gears of the feeding wheel sets feed both sides in the weft direction of the non-woven fabric into a location between the speed differential gears and the suction gears of the feeding wheel sets respectively along a warp direction;

In the feeding step 10, the fed non-woven fabric may be the non-woven fabric 10 as described above, therefore, the features and details of the non-woven fabric will not be described again.

In the wave forming step S20, the speed differential gears and suction gears engage and rotate with each other in a manner that the first teeth portions of the speed differential gears are inserted into the second groove portions of the suction gears and the second teeth portions of the suction gears are inserted into the first groove portions of the speed differential gears, such that both sides in the weft direction of the non-woven fabric respectively enter a location between the first teeth portions and the second groove portions and a location between the first groove portions and the second teeth portions, thereby forming regular wavy folds on the non-woven fabric along the warp direction.

In the fixing step S30, the suction gears and at least two pin chains in a form of conveyor belt are used to fix the wavy folds of the non-woven fabric, wherein a suction force is provided through the suction holes of the suction gears to make both sides in the weft direction of the non-woven fabric closely fit outer surfaces of the second teeth portions and the second groove portions of the suction gears, respectively, and the pin chains run in the form of conveyor belt while the suction gears rotate, making the pins puncture the non-woven fabric and enter the hollow grooves of the suction gears, respectively, to fix the wavy folds of the non-woven fabric; moreover, the suction gears stop providing the suction force after the pins puncture the non-woven fabric, such that the non-woven fabric can be smoothly transferred from the suction gears to the pin chains.

In the press-flattening step S40, the wavy folds of the non-woven fabric are press-flattened through at least two brush wheels, wherein the brush wheel rotates while the pin chains run in the form of conveyor belt, so as to press-flatten the wavy folds of the non-woven fabric on the pin chains.

In the preheating step S50, the pin chains are used to transport the non-woven fabric along the warp direction with maintaining a fixed distance in the weft direction of the pin chains, meanwhile, a heating device is used to heat the non-woven fabric to soften it.

In the broadening step S60, under proceeding the heating of the heating device, the pin chains are used to transport the softened non-woven fabric along the warp direction with the distance in the weft direction of the pin chains gradually increased to stretch the non-woven fabric in the weft direction, due to the stretching in the weft direction, a necking compensation effect of the non-woven fabric occurs along the warp direction due to the Poisson's ratio, thereby straightening the wavy folds that extend along the warp direction and are press-flattened, thereby making a fiber tissue of the non-woven fabric be oriented along the weft direction, such that the non-woven fabric is in a flat shape and has a stretching and restoring ability along the warp direction.

In the stabilizing step S70, under proceeding the heating of the heating device, the pin chains are used to transport the softened and stretched non-woven fabric along the warp direction with maintaining the increased distance in the weft direction of the pin chains for stabilizing the non-woven fabric.

In the cooling step S80, the stabilized non-woven fabric is cooled and set, thereby forming a non-woven fabric with elasticity in the warp direction.

In the manufacturing method of the non-woven fabric with elasticity in warp direction of the present invention, in the feeding step S10, the speed differential gears feed the non-woven fabric into the location between the speed differential gears and the suction gears along the warp direction at a speed higher than a conveying speed of the pin chains.

Preferably, the non-woven fabric with elasticity in warp direction of the present invention manufactured by the above equipment or the above method has an elongation in the warp direction between 50 and 350% (that is, he non-woven fabric can be stretched to a width in the warp direction 1.5 to 4.5 times of its natural width in the warp direction).

Preferably, in the above method, the suction holes are further provided on the second teeth portions.

Preferably, the heating temperature in the preheating step S50, the broadening step S60 and the stabilizing step S70 is 120 to 180°C, preferably 130 to 150°C.

Preferably, in the broadening step S60, a broadening ratio of the non-woven fabric 10 in the weft direction is between 15 and 100%.

Preferably, in the cooling step S80, the non-woven fabric 10 subjected to the stabilizing step S70 is cooled, for example, by air cooling or resting at room temperature, such that the non-woven fabric 10 returns to an unsoftened state, thereby fixing the shape of the non-woven fabric 10.

Preferably, in the fixing step S30, respective pins on the pin chains are aligned with a peak and/or a trough of the wavy folds of the non-woven fabric, respectively.

Preferably, in the above method, a ratio of a spacing between the first teeth portions, a spacing between the second teeth portions, and a spacing between the pins can be adjusted to 1:1:1 or 1:1:0.5.

Referring to FIGs. 11 and 12, the present invention provides a non-woven fabric with elasticity in warp direction 100, which can be manufactured by the above-mentioned manufacturing equipment or manufacturing method, and has the above-mentioned characteristics and technical effects.

Specifically, referring to FIG. 11, the non-woven fabric with elasticity in warp direction 100 of the present invention has a flat surface. Further, referring to FIG. 12, which shoes a partial enlarged view of a region a of FIG. 11, in which a fiber tissue 110 of the non-woven fabric with elasticity in warp direction 100 is substantially oriented in the weft direction.

When being stretched by an external force in the warp direction, since the fiber tissue 110 oriented in the weft direction of the non-woven fabric 100 can be stretched along the warp direction back to a state where the fiber orientation has not been altered, after the external force is stopped, the fiber tissue 110 of the non-woven fabric 100 will return to the state oriented along the weft direction, thereby the non-woven fabric 100 have the characteristics of high stretching and restoring characteristics in the warp direction that is superior to the elastic non-woven fabric of the prior art, that is, having high stretching and restoring ability.

In summary, the effects of the present invention are that: first, by feeding the non-woven fabric through the speed differential gears and the suction gears that engage with each other, regular wavy folds can be formed on the non-woven fabric, which is beneficial to ensure the surface flatness of the final elastic non-woven fabric; second, by providing a suction force through the suction gears to make the non-woven fabric closely fit outer surfaces of the teeth portions and groove portions of the suction gears, the non-woven fabric with the wavy folds can be transferred to the subsequent process with maintained shape, which is beneficial to improve the uniformity of the final fabric; third, by disposing a hollow groove at a center on the outer surfaces of the suction gears, a space for accommodating the pins on the pin chains after the pins puncture the non-woven fabric can be provided; fourth, by slightly stretching in the weft direction under heating to change the fiber orientation and subsequent cooling and setting, the non-woven fabric can have better elasticity in the warp direction than the prior art; fifth, by pre-forming regular wavy folds, the reduced area or reduced thickness of the non-woven fabric caused by necking during subsequent stretching can be compensated; sixth, by making the single-layerd non-woven fabric have excellent elasticity after processing, additional bonding materials or bonding steps can be omitted, thereby reducing the manufacturing costs and making the product thinner to improve comfort to user, and reducing the space and cost required for storage and transportation.

A person skilled in the art will understand that various modifications and changes can be made to the above embodiments, such as combinations, separations, substitutions, and changing configuration, without departing from the basic features of the present invention.

Therefore, the embodiments of the present invention are intended to illustrate the scope of the technical concept of the present invention, but the scope of the present invention is not limited by the above embodiments. Therefore, any modifications or changes to the present invention made under the same creative spirit should still be included in the scope to be protected of the present invention.

## Claims

1. A manufacturing method of a non-woven fabric with elasticity in warp direction (100), comprising:
a feeding step (S10), using at least two feeding wheel sets (F) to feed a non-woven fabric (10), wherein the feeding wheel sets (F) are respectively located at both sides in a weft direction (TD) of the non-woven fabric (10), and each feeding wheel set (F) includes a speed differential gear (20) and a suction gear (30) that engage with each other, wherein each speed differential gear (20) is provided with a plurality of first teeth portions (21) and a plurality of first groove portions (22) alternately arranged along an outer circumferential surface of the speed differential gear (20), and each suction gear (30) is provided with a hollow groove (34) at a center in the weft direction (TD) on an outer surface thereof, and each suction gear (30) is provided with a plurality of second teeth portions (31), a plurality of second groove portions (32) and a plurality of suction holes (33) at both sides in the weft direction (TD) of the hollow groove (34), respectively, wherein the second groove portions (32) and the second teeth portions (31) are alternately arranged along both sides in the weft direction (TD) of an outer circumferential surface of the suction gears (30), respectively, and the suction holes (33) are provided at least on the second groove portions (32), wherein the speed differential gears (20) feed both sides in the weft direction (TD) of the non-woven fabric (10) into a location between the speed differential gears (20) and the suction gears (30) respectively along a warp direction (MD);
a wave forming step (S20), rotating the speed differential gears (20) and the suction gears (30) with engaging with each other in a manner that the first teeth portions (21) are inserted into the second groove portions (32) and the second teeth portions (31) are inserted into the first groove portions (22), such that both sides in the weft direction (TD) of the non-woven fabric (10) respectively enter a location between the first teeth portions (21) and the second groove portions (32) and a location between the first groove portions (22) and the second teeth portions (31), thereby forming regular wavy folds on the non-woven fabric (10) along the warp direction (MD);
a fixing step (S30), using the suction gears (30) and at least two pin chains (40) in a form of conveyor belt to fix the wavy folds of the non-woven fabric (10), wherein the pin chains (40) are respectively located on both sides in the weft direction (TD) of the non-woven fabric (10), and the feeding wheel sets (F) are respectively arranged above the pin chains (40), and a plurality of pins (41) are provided on each pin chain (40), wherein a suction force is provided through the suction holes (33) to make both sides in the weft direction (TD) of the non-woven fabric (10) closely fit outer surfaces of the second teeth portions (31) and the second groove portions (32), respectively, and the pin chains (40) run in the form of conveyor belt while the suction gears (30) rotate, making the pins (41) puncture the non-woven fabric (10) and enter the hollow grooves (34), respectively, to fix the wavy folds of the non-woven fabric (10), and the suction gears (30) stop providing the suction force after the pins (41) puncture the fed non-woven fabric (10), such that the non-woven fabric (10) can be smoothly transferred from the suction gears (30) to the pin chains (40);
a press-flattening step (S40), press-flattening the wavy folds of the non-woven fabric (10) through at least two brush wheels (50), wherein the brush wheels (50) are respectively disposed above the pin chains (40) at downstream in the warp direction (MD) of the feeding wheel sets (F), and the brush wheels (50) rotate while the pin chains (40) run in the form of conveyor belt, so as to press-flatten the wavy folds of the non-woven fabric (10) on the pin chains (40);
a preheating step (S50), using the pin chains (40) to transport the non-woven fabric (10) along the warp direction (MD) with maintaining a fixed distance in the weft direction (TD) of the pin chains (40), meanwhile, using a heating device (60) to heat the non-woven fabric (10) to soften it;
a broadening step (S60), under proceeding the heating of the heating device (60), using the pin chains (40) to transport the softened non-woven fabric (10) along the warp direction (MD) with the distance in the weft direction (TD) of the pin chains (40) gradually increased to stretch the non-woven fabric (10) in the weft direction (TD), such that a necking compensation effect of the non-woven fabric (10) occurs along the warp direction (MD) to straighten the wavy folds that extend along the warp direction (MD) and are press-flattened, thereby making a fiber tissue of the non-woven fabric (10) be oriented along the weft direction (TD), such that the non-woven fabric (10) is in a flat shape and has a stretching and restoring ability along the warp direction (MD);
a stabilizing step (S70), under proceeding the heating of the heating device (60), using the pin chains (40) to transport the softened and stretched non-woven fabric (10) along the warp direction (MD) with maintaining the increased distance in the weft direction (TD) for stabilizing the non-woven fabric (10); and
a cooling step (S80), cooling the stabilized non-woven fabric (10) to set it, thereby forming a non-woven fabric with elasticity in the warp direction (100);
wherein in the feeding step (S10), the speed differential gears (20) feed the non-woven fabric (10) into the location between the speed differential gears (20) and the suction gears (30) along the warp direction (MD) at a speed higher than a conveying speed of the pin chains (40).

2. The manufacturing method according to claim 1, wherein the suction holes (33) are further provided on the second teeth portions (31).

3. The manufacturing method according to claim 1, wherein the heating temperature in the preheating step (S50), the broadening step (S60) and the stabilizing step (S70) is 120 to 180°C.

4. The manufacturing method according to claim 1, wherein in the broadening step (S60), a broadening ratio of the non-woven fabric (10) in the weft direction (TD) is between 15 and 100%.

5. The manufacturing method according to claim 1, wherein in the fixing step (S30), respective pins (41) on the pin chains (40) are aligned with a peak and/or a trough of the wavy folds, respectively.

6. The manufacturing method according to claim 1, wherein a ratio of a spacing between the first teeth portions (21), a spacing between the second teeth portions (31), and a spacing between the pins (41) is 1:1:1 or 1:1:0.5.

7. The manufacturing method according to claim 1, wherein the non-woven fabric (10) is made by spun-bonding, spunlace, thermal-bonding, melt-blowing, or needle-punching.

8. The manufacturing method according to claim 1, wherein the non-woven fabric (10) is made of a material selected from a group consisting of PP, PE, PET, PP/PE, PP/PET, or a combination thereof.

9. A non-woven fabric with elasticity in warp direction (100) manufactured according to the manufacturing method of claim 1, wherein
the non-woven fabric with elasticity in warp direction (100) has a flat surface and has a fiber tissue (110) substantially oriented in the weft direction (TD), such that the non-woven fabric with elasticity in warp direction (100) has a stretching and restoring ability along the warp direction (MD).

10. The non-woven fabric with elasticity in warp direction (100) according to claim 9, wherein the non-woven fabric with elasticity in warp direction (100) has an elongation in the warp direction (MD) between 50 and 350%.

## Patentansprüche

1. Verfahren zur Herstellung eines Vliesstoffs mit Elastizität in Kettrichtung (100), umfassend:
einen Zuführschritt (S10), bei dem mindestens zwei Zuführradsätze (F) verwendet werden, um ein Vlies (10) zuzuführen, wobei die Zuführradsätze (F) jeweils an beiden Seiten in Schussrichtung (TD) des Vlieses (10) angeordnet sind und jeder Zuführradsatz (F) ein Differentialgetriebe (20) und ein Saugrad (30) umfasst, die miteinander in Eingriff stehen, wobei jedes Differentialgetriebe (20) mit einer Vielzahl von ersten Zahnabschnitten (21) und einer Vielzahl von ersten Nutabschnitten (22) versehen ist, die abwechselnd entlang einer Außenumfangsfläche des Differentialgetriebes (20) angeordnet sind, und jedes Saugzahnrad (30) an einer Mitte in Schussrichtung (TD) auf seiner Außenfläche mit einer hohlen Nut (34) versehen ist, und jedes Saugzahnrad (30) mit einer Vielzahl von zweiten Zahnabschnitten (31), einer Vielzahl von zweiten Nutabschnitten (32) und einer Vielzahl von Sauglöchern (33) jeweils an beiden Seiten in Schussrichtung (TD) der hohlen Nut (34), wobei die zweiten Nutabschnitte (32) und die zweiten Zahnabschnitte (31) abwechselnd entlang beider Seiten in Schussrichtung (TD) einer Außenumfangsfläche der Saugzahnräder (30) angeordnet sind und die Sauglöcher (33) zumindest an den zweiten Nutabschnitten (32) vorgesehen sind, wobei die Geschwindigkeitsdifferenzgetriebe (20) beide Seiten in Schussrichtung (TD) des Vliesstoffs (10) entlang einer Kettrichtung (MD) jeweils in einen Bereich zwischen den Geschwindigkeitsdifferenzgetrieben (20) und den Saugzahnrädern (30) einführen;
ein Wellenbildungsschritt (S20), bei dem die Geschwindigkeitsdifferenzgetriebe (20) und die Saugzahnräder (30) in Eingriff miteinander gedreht werden, derart, dass die ersten Zahnabschnitte (21) in die zweiten Nutabschnitte (32) und die zweiten Zahnabschnitte (31) in die ersten Nutabschnitte (22) eingeführt werden, sodass beide Seiten des Vliesstoffs (10) in Schussrichtung (TD) jeweils in eine Position zwischen den ersten Zahnabschnitten (21) und den zweiten Nutabschnitten (32) sowie in eine Position zwischen den ersten Nutabschnitten (22) und den zweiten Zahnabschnitten (31) gelangen, wodurch regelmäßige wellenförmige Falten auf dem Vliesstoff (10) entlang der Kettrichtung (MD) gebildet werden;
einen Fixierschritt (S30), bei dem die Saugzahnräder (30) und mindestens zwei Stiftketten (40) in Form eines Förderbandes verwendet werden, um die wellenförmigen Falten des Vliesstoffs (10) zu fixieren, wobei die Stiftketten (40) jeweils auf beiden Seiten in Schussrichtung (TD) des Vliesstoffs (10) angeordnet sind und die ZuführradSätze (F) jeweils über den Stiftketten (40) angeordnet sind, und an jeder Stiftkette (40) eine Vielzahl von Stiften (41) vorgesehen ist, wobei durch die Sauglöcher (33) eine Saugkraft bereitgestellt wird, um beide Seiten in Schussrichtung (TD) des Vliesstoffs (10) eng an die Außenflächen der zweiten Zahnabschnitte (31) bzw. der zweiten Nutabschnitte (32) eng anliegen, und die Stiftkette (40) in Form eines Förderbandes läuft, während sich die Saugzahnräder (30) drehen, wodurch die Stifte (41) das Vlies (10) durchstechen und jeweils in die hohlen Nuten (34) eindringen, um die wellenförmigen Falten des Vlieses (10) zu fixieren, und die Saugzahnräder (30) stellen die Saugkraft ein, nachdem die Stifte (41) das zugeführte Vlies (10) durchstoßen haben, so dass das Vlies (10) reibungslos von den Saugzahnrädern (30) auf die Stiftketten (40) übertragen werden kann;
einen Glättungsschritt (S40), bei dem die wellenförmigen Falten des Vliesstoffs (10) durch mindestens zwei Bürstenräder (50) geglättet werden, wobei die Bürstenräder (50) jeweils oberhalb der Stiftketten (40) stromabwärts in Kettrichtung (MD) der Zuführradgruppen (F) angeordnet sind und sich die Bürstenräder (50) drehen, während die Stiftketten (40) in Form eines Förderbandes laufen, um die wellenförmigen Falten des Vliesstoffs (10) auf den Stiftketten (40) zu glätten;
einen Vorheizschritt (S50), bei dem die Stiftketten (40) verwendet werden, um das Vlies (10) entlang der Kettrichtung (MD) unter Beibehaltung eines festen Abstands in der Schussrichtung (TD) der Stiftketten (40) zu transportieren, während gleichzeitig eine Heizeinrichtung (60) verwendet wird, um das Vlies (10) zu erwärmen und es weich zu machen;
einen Breitmachschritt (S60), bei dem unter Fortsetzung der Erwärmung durch die Heizvorrichtung (60) das erweichte Vlies (10) mit Hilfe der Stiftkette (40) entlang der Kettrichtung (MD) transportiert wird, wobei der Abstand der Stiftkette (40) in Schussrichtung (TD) allmählich vergrößert wird, um das Vlies (10) in Schussrichtung (TD) gestreckt wird, so dass ein Einengungskompensationseffekt des Vliesstoffs (10) entlang der Kettrichtung (MD) auftritt, um die wellenförmigen Falten, die sich entlang der Kettrichtung (MD) erstrecken und durch Pressen abgeflacht werden, zu glätten, wodurch ein Faserverzweigungsgeflecht des Vliesstoffs (10) entlang der Schussrichtung (TD) ausgerichtet wird, so dass der Vliesstoff (10) eine flache Form aufweist und eine Dehnungs- und Rückstellfähigkeit entlang der Kettrichtung (MD) besitzt;
einen Stabilisierungsschritt (S70), bei dem unter Fortsetzung der Erwärmung durch die Heizvorrichtung (60) die Stiftkette (40) verwendet wird, um das erweichte und gedehnte Vlies (10) entlang der Kettrichtung (MD) zu transportieren, wobei der vergrößerte Abstand in der Schussrichtung (TD) beibehalten wird, um das Vlies (10) zu stabilisieren; und
einen Kühlschritt (S80), bei dem das stabilisierte Vlies (10) gekühlt wird, um es zu fixieren, wodurch ein Vlies mit Elastizität in Kettrichtung (100) gebildet wird;
wobei im Zuführschritt (S10) die Geschwindigkeitsdifferenzräder (20) das Vlies (10) entlang der Kettrichtung (MD) mit einer Geschwindigkeit, die höher ist als eine Fördergeschwindigkeit der Stiftketten (40), in den Bereich zwischen den Geschwindigkeitsdifferenzrädern (20) und den Saugrädern (30) zuführen.

2. Herstellungsverfahren nach Anspruch 1, wobei die Sauglöcher (33) ferner an den zweiten Zahnabschnitten (31) vorgesehen sind.

3. Verfahren gemäß Anspruch 1, wobei die Erwärmungstemperatur im Vorwärmschritt (S50), im Breitlegungsschritt (S60) und im Stabilisierungsschritt (S70) 120 bis 180 °C beträgt.

4. Verfahren gemäß Anspruch 1, wobei im Breitstreckungsschritt (S60) ein Breitstreckungsverhältnis des Vliesstoffs (10) in Schussrichtung (TD) zwischen 15 und 100 % liegt.

5. Verfahren gemäß Anspruch 1, wobei im Fixierschritt (S30) jeweilige Stifte (41) an den Stiftketten (40) jeweils mit einem Scheitel und/oder einem Tal der wellenförmigen Falten ausgerichtet werden.

6. Verfahren zur Herstellung nach Anspruch 1, wobei das Verhältnis des Abstands zwischen den ersten Zahnabschnitten (21), des Abstands zwischen den zweiten Zahnabschnitten (31) und des Abstands zwischen den Stiften (41) 1:1:1 oder 1:1:0,5 beträgt.

7. Verfahren zur Herstellung nach Anspruch 1, wobei das Vlies (10) durch Spinnvliesverfahren, Spunlace-Verfahren, Thermobonding, Schmelzblasverfahren oder Nadelvliesverfahren hergestellt wird.

8. Verfahren zur Herstellung nach Anspruch 1, wobei das Vlies (10) aus einem Material hergestellt ist, das aus einer Gruppe ausgewählt ist, die aus PP, PE, PET, PP/PE, PP/PET oder einer Kombination davon besteht.

9. Ein Vliesstoff mit Elastizität in Kettrichtung (100), hergestellt gemäß dem Herstellungsverfahren nach Anspruch 1, wobei
der Vliesstoff mit Elastizität in Kettrichtung (100) eine flache Oberfläche aufweist und ein Faservlies (110) aufweist, das im Wesentlichen in Schussrichtung (TD) ausgerichtet ist, so dass der Vliesstoff mit Elastizität in Kettrichtung (100) eine Dehnungs- und Rückstellfähigkeit entlang der Kettrichtung (MD) aufweist.

10. Vliesstoff mit Elastizität in Kettrichtung (100) gemäß Anspruch 9, wobei der Vliesstoff mit Elastizität in Kettrichtung (100) eine Dehnung in Kettrichtung (MD) zwischen 50 und 350 % aufweist.

## Revendications

1. Procédé de fabrication d'un tissu non tissé présentant une élasticité dans le sens de la chaîne (100), comprenant:
une étape d'alimentation (S10), utilisant au moins deux ensembles de roues d'alimentation (F) pour alimenter un tissu non tissé (10), dans laquelle les ensembles de roues d'alimentation (F) sont respectivement situés de part et d'autre dans une direction de trame (TD) du tissu non tissé (10), et chaque ensemble de roues d'alimentation (F) comprend un engrenage différentiel (20) et un engrenage d'aspiration (30) qui s'engrènent l'un avec l'autre, dans lequel chaque engrenage différentiel (20) est muni d'une pluralité de premières parties dentées (21) et d'une pluralité de premières parties rainurées (22) disposées en alternance le long d'une surface circonférentielle extérieure de l'engrenage différentiel (20), et chaque pignon d'aspiration (30) est muni d'une rainure creuse (34) au centre dans la direction de la trame (TD) sur sa surface extérieure, et chaque pignon d'aspiration (30) est muni d'une pluralité de secondes parties dentées (31), une pluralité de secondes parties de rainure (32) et une pluralité de trous d'aspiration (33) situés respectivement de part et d'autre dans la direction de la trame (TD) de la rainure creuse (34), les secondes parties de rainure (32) et les secondes parties dentées (31) étant disposées en alternance le long des deux côtés dans la direction de la trame (TD) d'une surface circonférentielle extérieure des engrenages d'aspiration (30), respectivement, et les trous d'aspiration (33) sont prévus au moins sur les secondes parties de rainure (32), dans lequel les engrenages à différence de vitesse (20) acheminent les deux côtés dans la direction de la trame (TD) du non-tissé (10) vers un emplacement situé entre les engrenages à différence de vitesse (20) et les engrenages d'aspiration (30), respectivement, le long d'une direction de la chaîne (MD);
une étape de formation d'ondulations (S20), consistant à faire tourner les engrenages à différence de vitesse (20) et les engrenages d'aspiration (30) en les mettant en prise les uns avec les autres de manière à ce que les parties dentées (21) s'insèrent dans les secondes parties de rainure (32) et les secondes parties dentées (31) s'insèrent dans les premières parties de rainure (22), de sorte que les deux côtés dans la direction de la trame (TD) du non-tissé (10) pénètrent respectivement dans un endroit situé entre les premières parties dentées (21) et les secondes parties rainurées (32) et dans un endroit situé entre les premières parties rainurées (22) et les secondes parties dentées (31), formant ainsi des plis ondulés réguliers sur le non-tissé (10) le long de la direction de la chaîne (MD);
une étape de fixation (S30), utilisant les engrenages d'aspiration (30) et au moins deux chaînes à broches (40) sous forme d'une bande transporteuse pour fixer les plis ondulés du tissu non tissé (10), dans laquelle les chaînes à broches (40) sont respectivement situées de part et d'autre dans la direction de la trame (TD) du tissu non tissé (10), et les ensembles de roues d'alimentation (F) sont respectivement disposés au-dessus des chaînes à broches (40), et une pluralité de broches (41) sont prévues sur chaque chaîne à broches (40), dans lequel une force d'aspiration est fournie par les orifices d'aspiration (33) pour amener les deux côtés dans la direction de la trame (TD) du non-tissé (10) à épouser étroitement les surfaces extérieures des secondes parties dentées (31) et des secondes parties rainurées (32), respectivement, et les chaînes à broches (40) se déplacent sous la forme d'une bande transporteuse tandis que les engrenages d'aspiration (30) tournent, ce qui fait que les broches (41) perforent le tissu non tissé (10) et pénètrent dans les rainures creuses (34), respectivement, pour fixer les plis ondulés du tissu non tissé (10), et les engrenages d'aspiration (30) cessent de fournir la force d'aspiration une fois que les broches (41) ont perforé le tissu non tissé (10) acheminé, de sorte que le tissu non tissé (10) puisse être transféré en douceur des engrenages d'aspiration (30) vers les chaînes à broches (40);
une étape d'aplatissement par pression (S40), consistant à aplatir par pression les plis ondulés du tissu non tissé (10) à l'aide d'au moins deux roues à brosses (50), dans laquelle les roues à brosses (50) sont respectivement disposées au-dessus des chaînes à broches (40) en aval dans le sens de la chaîne (MD) des ensembles de roues d'alimentation (F), et les roues à brosses (50) tournent tandis que les chaînes à broches (40) fonctionnent à la manière d'une bande transporteuse, de manière à aplatir par pression les plis ondulés du tissu non tissé (10) sur les chaînes à broches (40);
une étape de préchauffage (S50), consistant à utiliser les chaînes à broches (40) pour transporter le non-tissé (10) dans le sens de la chaîne (MD) tout en maintenant une distance fixe dans le sens de la trame (TD) des chaînes à broches (40), tout en utilisant un dispositif de chauffage (60) pour chauffer le non-tissé (10) afin de le ramollir;
une étape d'élargissement (S60), tout en poursuivant le chauffage par le dispositif de chauffage (60), consistant à utiliser les chaînes à broches (40) pour transporter le tissu non tissé ramolli (10) dans le sens de la chaîne (MD) tout en augmentant progressivement la distance dans le sens de la trame (TD) des chaînes à broches (40) afin d'étirer le tissu non tissé (10) dans le sens de la trame (TD), de telle sorte qu'un effet de compensation du rétrécissement du tissu non tissé (10) se produit le long de la direction de la chaîne (MD) pour redresser les plis ondulés qui s'étendent le long de la direction de la chaîne (MD) et sont aplatis par pression, ce qui fait que le tissu fibreux du non-tissé (10) s'oriente dans le sens de la trame (TD), de sorte que le non-tissé (10) présente une forme plate et possède une capacité d'étirement et de retour élastique dans le sens de la chaîne (MD);
une étape de stabilisation (S70), pendant le chauffage du dispositif de chauffage (60), consistant à utiliser les chaînes à broches (40) pour transporter le tissu non tissé (10) ramolli et étiré dans le sens de la chaîne (MD) tout en maintenant la distance accrue dans le sens de la trame (TD) afin de stabiliser le tissu non tissé (10); et
une étape de refroidissement (S80), consistant à refroidir le non-tissé stabilisé (10) pour le fixer, formant ainsi un non-tissé présentant une élasticité dans la direction de la chaîne (100);
dans lequel, lors de l'étape d'alimentation (S10), les engrenages à différence de vitesse (20) acheminent le tissu non tissé (10) vers l'emplacement situé entre les engrenages à différence de vitesse (20) et les engrenages d'aspiration (30) le long de la direction de la chaîne (MD) à une vitesse supérieure à la vitesse de transport des chaînes à broches (40).

2. Procédé de fabrication selon la revendication 1, dans lequel les orifices d'aspiration (33) sont en outre prévus sur les secondes parties dentées (31).

3. Procédé de fabrication selon la revendication 1, dans lequel la température de chauffage lors de l'étape de préchauffage (S50), de l'étape d'élargissement (S60) et de l'étape de stabilisation (S70) est comprise entre 120 et 180 °C.

4. Procédé de fabrication selon la revendication 1, dans lequel, lors de l'étape d'élargissement (S60), le taux d'élargissement du non-tissé (10) dans la direction de la trame (TD) est compris entre 15 et 100 %.

5. Procédé de fabrication selon la revendication 1, dans lequel, lors de l'étape de fixation (S30), les broches respectives (41) sur les chaînes de broches (40) sont alignées respectivement avec un sommet et/ou un creux des plis ondulés.

6. Procédé de fabrication selon la revendication 1, dans lequel le rapport entre l'espacement entre les premières parties en dents (21), l'espacement entre les secondes parties en dents (31) et l'espacement entre les broches (41) est de 1:1:1 ou 1:1:0,5.

7. Procédé de fabrication selon la revendication 1, dans lequel le tissu non tissé (10) est fabriqué par filage-liage, filage-enchevêtrement, thermoliage, soufflage à l'état fondu ou aiguilletage.

8. Procédé de fabrication selon la revendication 1, dans lequel le tissu non tissé (10) est constitué d'un matériau choisi parmi un groupe comprenant le PP, le PE, le PET, le PP/PE, le PP/PET ou une combinaison de ceux-ci.

9. Tissu non tissé présentant une élasticité dans le sens de la chaîne (100) fabriqué selon le procédé de fabrication de la revendication 1, dans lequel
le tissu non tissé présentant une élasticité dans le sens de la chaîne (100) présente une surface plane et comporte un tissu de fibres (110) orienté sensiblement dans le sens de la trame (TD), de telle sorte que le tissu non tissé présentant une élasticité dans le sens de la chaîne (100) présente une capacité d'étirement et de retour élastique le long du sens de la chaîne (MD).

10. Tissu non tissé présentant une élasticité dans le sens de la chaîne (100) selon la revendication 9, dans lequel le tissu non tissé présentant une élasticité dans le sens de la chaîne (100) présente un allongement dans le sens de la chaîne (MD) compris entre 50 et 350 %.
